

Dec. 14, 1937.

W. W. ROWE

2,101,874

COMPOSITE FABRIC

Filed March 8, 1934



INVENTOR,  
*William Wallace Rowe*

BY  
*Allen & Allen*

ATTORNEYS

## UNITED STATES PATENT OFFICE

2,101,874

## COMPOSITE FABRIC

William Wallace Rowe, Cincinnati, Ohio, assignor to The Paper Service Company, Lockland, Ohio, a corporation of Ohio

Application March 8, 1934, Serial No. 714,647

12 Claims. (Cl. 154—50)

My invention relates to specialized composite fabrics. These fabrics, as will be readily understood, are available for many uses, and in the formation of many different types of articles.

5 In the ensuing specifications I shall describe them with particular reference to the manufacture of bags, wherein arise a number of the problems in the solution of which my invention has an especial application. It will be understood, however, 10 that this particular use is exemplary only, and is not limiting in any degree.

The fundamental object of my invention is the provision of a composite fabric of proofed character, and in particular of waterproofed character, with certain other attendant advantages 15 which will hereinafter be clear.

This and the other objects of my invention which will be set forth hereinafter, or will be apparent to one skilled in the art upon reading these 20 specifications, I accomplish in those structures of which I shall hereinafter set forth certain exemplary embodiments. A drawing forms part of these specifications, wherein I have shown in somewhat magnified and exaggerated form, a 25 cross-section of an exemplary fabric embodying my invention.

Hitherto bags for heavy duty, as well as a number of other articles, have been made from a composite fabric in which creped paper is cemented 30 to a textile material such, for example, as burlap or cotton. While other adhesives have been used, the one most commonly employed is asphalt. There is a growing use for bags and other containers for the shipment either of hydroscopic 35 materials or materials which will be damaged by moisture, air or other gases. Likewise there is a growing use for composite materials of this character in other articles or constructions wherein either the retention or the exclusion of 40 water, moisture, gases, and the like, is essential. There has been considerable development in the formation of seam or joint structures which are in themselves more highly resistant to penetration than seam or joint structures which have 45 been in current use in the art; but no proofed seam or joint will be effective in producing, for example, a waterproof article, unless the fabric itself, of which such article is made, is proofed against water or other deleterious influence.

50 Consequently, there is great need in the industry for the development of truly proofed fabrics.

It must be remembered that in constructions of this character, the fabric is liable to strains which tend to distort it in various directions. 55 Thus, in a bag subject to ordinary handling, the

textile material is bent and bulged, as well as stretched along the diagonal. Likewise, the creped paper layer is distorted, and the asphaltic layer between them is subject to disrupting strains. Even assuming, therefore, that the asphaltic layer were absolutely continuous, and did render the fabric waterproof as initially formed, these disrupting strains speedily operate to destroy the proofed character of the fabric. Thus, 10 in a bag of ordinary construction, proofing tests applied after the bag has been in use, always show a very marked and very considerable loss of resistance as compared to tests before use. Several factors are of importance here. Normally 15 the asphalt employed must be of a fairly hard type. In bags of the character referred to, the paper is disposed inwardly, with the cloth lying on the outside of the container. The use of soft asphalt would be productive of a staining of the burlap or other textile fabric; and under conditions of heat, as in warm climates, or when bags 20 are filled with hot materials, the asphalt would strike entirely through the cloth and serve to stick adjacent containers together, as well as to render the containers very unsightly. This is true 25 as well of thick layers of the normally used and relatively hard asphaltic substances, as of layers of softer substance.

So far as proofness is concerned, the advantage, 30 however, lies with layers of softer asphalt, bitumen or other adhesive, because even thick layers of hard adhesive can quite readily be cracked and disrupted by the strains aforesaid, whereas softer layers, retaining a more or less continuous plasticity, not only give under such strains without disrupting, but if disrupted, can seal themselves in a new formation without altering the proofed character of the fabric. Softer bitumens, 35 however, have the additional disadvantage of staining through the paper on the inside of the bag or container, so that the containers are rendered unsightly, and are not acceptable to the general public, for example, as containers for food stuffs or the like.

In the practice of my invention, I provide a construction 45 wherein a paper layer is cemented to a layer of textile fabric with a relatively thin layer of adhesive and/or a non-staining character of adhesive. I provide a second paper layer displaced from the first, and I confine therebetween a 50 layer of proofing substance, preferably of relatively soft character, and preferably also having a continuous resident plasticity as aforesaid. Since this layer is confined between layers of paper, it is 55 prevented from coming through the textile layer.

Additionally, either layer of paper may be treated in such a way as to prevent the softer layer of adhesive, if it has staining characteristics, from staining through said layer.

5 I shall now describe in detail, an exemplary embodiment of my invention and certain modifications thereof; and for clearness, reference is now made to the drawing, wherein A represents a layer of cloth, such as burlap, Osnaburg, cotton 10 scrim, or other fabric, without limitation, and including unwoven material, such as crossed cords or the like. A layer of creped paper B is cemented to the layer A by means of an adhesive C. The adhesive C may be any desired, including, but 15 without limitation, rubber latex, glues, vegetable pastes, bitumens and the like. Particularly if the layer C is of bitumen or other staining adhesive, or of an adhesive which would tend to become soft under the influence of any condition to which the 20 fabric might be subjected in use, and to come through the textile layer, the layer C should be relatively thin. Aside from its moisture-proofing value, its function is, of course, to adhere together the textile layer and the other layers of my 25 composite fabric, and this function may be of importance only until the final article has been constructed therefrom, or may be of importance in maintaining a continuously adhered condition throughout the life of the article. In the manu- 30 facture of bags, for example, where the inner layers, comprising paper and adhesives, have the qualities of universal stretchability, it is not necessary to maintain adhesion between the textile and the other layers throughout the life of the article.

35 While I prefer to make my layer of creped paper B, in accordance with the teachings of my Re-issue Patent No. 17,633, i. e. by creping the paper by means of the positive adhesive action of a thermoplastic substance, such as asphalt, and 40 while I also prefer to give the paper the qualities of universal stretchability, in accordance with the teachings of the co-pending application of William C. Kemp, Serial No. 626,059, filed July 29, 1932, i. e. by creping the paper twice upon the 45 diagonal, the different sets of creping crinkles crossing each other, yet such products and methods are not a limitation upon my present invention. Where the paper is creped by means of a thermoplastic, I may, for example, but again 50 without limitation, use a high melting point asphalt, say of approximately 180° F., as obtained by the A. S. T. M. standard test. I may also use the asphalt so applied to cement the paper to the burlap or the like A, the asphalt in this case con- 55 stituting the layer marked C. This, again, is not a limitation upon my invention; but I may take the same paper webs or other webs otherwise produced, and cement them to the layer A by any procedure desired.

60 I have shown another layer of paper D dis- placed from the first layer, and having therebetween an adhesive substance or substances indicated generally at E. Preferably a part, at least, of such layer or layers comprises a proofing sub- 65 stance. Where asphalt or other bitumen is em- ployed, this proofing layer preferably will have a relatively permanent plasticity at normal tem- peratures, and may be of an asphaltic substance of lower melting point, say around 105-115° F., 70 as determined by the standard test referred to above. The layer may, however, be of other proofing substances, as set forth above.

Particularly where asphalt or other bitumen is used of fairly low melting point, it may be ad- 75 visable to coat at least the upper layer of paper

D where it comes thereagainst, with a substance which will prevent the staining of the ply D, by absorption of the lighter constituents of the softer coating. This proofing coat may be of any substance desired, including, but without limitation, 5 a rubber latex; but I have found that it is sufficient to provide the sheet D with a coating of harder asphalt similar to the harder coating described above. Therefore, in my drawing I have subdivided the layer E into a layer F of soft 10 asphalt, and a layer G of harder asphalt compara- 15 ble to the layer C. Where the paper web D is creped by means of an asphaltic substance, the layer G may comprise or consist wholly of the adhesive used in the creping step. 15

It will be noted that the softer layer F is, in my construction, sealed between layers D and B. It may tend to be absorbed, in more or less degree, by the layer B; but this is of no consequence, so far as appearance is concerned, the layer B being 20 an interior ply, and even is of assistance in the proofing, in that it becomes less likely for moisture to pass through a defect in the layer C, and then travel in the paper layer B until it can find another defect through which it can pass into 25 the interior of the bag or container made of my composite fabric. In order to prevent staining, where desired, it is also possible to employ paper layers having at least one surface formed of hard 30 sized fibers or the like. 30

The manner of combining the various layers which go to make up my composite fabric, is not a limitation upon my invention. So long as a good bond is obtained, the paper layers may be assembled together and afterwards joined to 35 the textile or other material, or one layer can first be joined to the textile and the other layer added with the interposition of the intervening coat or coats. It is likewise possible to use two 40 medium melting point layers as layers G and F, but this is ordinarily not to be preferred, excepting that a double coating, where the coatings are relatively thin, has been found in practice to give a much more water- and moisture-proof article 45 than a single coating would give. This is because a single coating may have a tendency either to be imperfect, or to be cracked or broken, whereas, when two or more coatings are used between the 50 layers of paper, the second and/or additional coats serve to seal imperfections in the first. The 55 purpose of using a low melting point sealing layer, such as F, is to provide in the bag a layer which will not be subject to brittleness, and therefore will not tend to lose its proofing character when the composite fabric is subject to use. Resilient plasticity, while desirable for the self-sealing 60 feature which it has, is not a limitation upon my invention. I may employ, if I choose, a layer of substance which is proof, but which is elastic 65 and resilient, and does not become hard and brittle under the influence of temperature changes or other influences to which the fabric may be subjected. There is also a tendency in plastic layers, such as low melting point asphalts, to amalgamate somewhat with higher melting point 70 layers, and to seal cracks therein as and when they are formed.

It will be understood that my invention is not limited to the specific embodiment which I have chosen, and not only that modifications may be made therein without departing from the spirit 75 of my invention, but that additions may be made to such composite fabric also without such departure. There may be more than two paper layers, and/or the textile layer A may be faced on its 75

outer side with paper or other material as may be desired, by way of example. I have illustrated in my drawing, in a diagrammatic way, the general features of my invention, and what I claim 5 as new and desire to secure by Letters Patent, is:—

1. A composite fabric comprising in the order named, a layer of cloth, a layer of adhesive, a layer of creped paper, a plurality of layers of 10 adhesive, and a layer of creped paper.

2. The product as claimed in claim 1, in which the paper layers have the characteristic of universal stretchability.

3. A composite fabric comprising in the order 15 named, a layer of cloth, a layer of high melting point asphalt, a layer of paper, at least one layer of low melting point asphalt, a layer of high melting point asphalt, and a layer of paper.

4. A composite fabric comprising in the order 20 named, a layer of paper, a sealing substance, a non-brittle proofing substance, and a layer of paper, the said composite fabric being joined, as such, to a layer of cloth.

5. A composite fabric comprising a layer of 25 cloth, a layer of paper creped by means of a thermoplastic adhesive and joined by said adhesive to said cloth, a layer of non-brittle proofing substance overlying said paper layer, and a second layer of paper creped by means of a thermoplastic adhesive, so disposed on said proofing layer that the resident film of said thermoplastic adhesive on said last mentioned paper layer lies 30 against said proofing layer.

6. A composite fabric comprising at least two 35 layers of paper and a plurality of layers of cementitious substances located therebetween, one of said layers of cementitious substance being bitumen, and at least one other layer of cementitious substance being rubber derived from latex, said last mentioned layer lying adjacent one of said paper layers.

7. A composite fabric comprising at least two 40 layers of paper and a plurality of layers of cementitious substances located therebetween, one of said layers of cementitious substance being a layer of rubber derived from latex, and at least one other of said layers of cementitious sub-

stance being a layer of bituminous material, said layer of bituminous material lying between a paper face of said composite fabric and said layer of rubber derived from latex.

8. A composite fabric comprising two layers of 5 paper and a plurality of layers of cementitious substances located therebetween, one of said layers, at least, being a layer of a staining adhesive, and one other of said layers, at least, being a layer of non-staining adhesive located between said layer of staining adhesive and one of said paper faces, said last mentioned paper face, at least, consisting of a layer of paper which is stretchable in 10 all directions.

9. A composite fabric comprising cloth, a plurality of layers of paper lying on the same side of said cloth, one of which is in adhesive union therewith, a layer of staining adhesive between at least an adjacent pair of said paper layers, and a coating of stain preventing substance associated with at least the outer one of said paper 20 layers.

10. A composite fabric comprising a plurality of contiguous paper layers and a layer of cloth, 25 one of said paper layers being joined to said cloth by a layer of bituminous adhesive, and a layer of bituminous adhesive disposed between said paper layers, the first mentioned bituminous layer being brittle at a temperature of use at which temperature the second mentioned of said bituminous 30 layers is non-brittle.

11. The product as claimed in claim 3 in which the layer of low melting point asphalt is at least 35 partially absorbed into the intermediate layer of paper.

12. A composite fabric comprising two layers of paper and a plurality of layers of cementitious substance located therebetween, one of said layers at least being a layer of low melting point asphalt and another of said layers at least being a layer of high melting point asphalt located between said layer of low melting point asphalt and one of said paper faces, said last mentioned paper face at least consisting of a layer of paper which is stretchable in all directions. 40 45

WILLIAM WALLACE ROWE.